

# United States Patent [19]

Barber

[11] Patent Number: 4,737,341

[45] Date of Patent: Apr. 12, 1988

[54] TITANIUM-BASE ALLOYS

[75] Inventor: Anthony C. Barber, Sutton, England

[73] Assignee: IMI Titanium Limited, Wilton,  
United Kingdom

[21] Appl. No.: 38,353

[22] Filed: Apr. 14, 1987

[30] Foreign Application Priority Data

Apr. 18, 1986 [GB] United Kingdom ..... 8609580

[51] Int. Cl.<sup>4</sup> ..... C22C 14/00

[52] U.S. Cl. ..... 420/419; 420/418

[58] Field of Search ..... 420/418, 419, 421;  
148/12.7 B, 407, 421

[56] References Cited

U.S. PATENT DOCUMENTS

3,540,946 11/1970 Minton et al. ..... 420/418

FOREIGN PATENT DOCUMENTS

596202 4/1960 Canada ..... 420/418

1403206 8/1975 United Kingdom .

Primary Examiner—L. Dewayne Rutledge

Assistant Examiner—Robert L. McDowell

Attorney, Agent, or Firm—Cushman, Darby & Cushman

[57]

ABSTRACT

Creep resistant titanium alloys containing aluminum, zirconium, molybdenum and germanium plus optional silicon, carbon, tin and niobium.

9 Claims, No Drawings

## TITANIUM-BASE ALLOYS

## BACKGROUND OF THE INVENTION

This invention relates to titanium base alloys. All percentages are weight percentages.

## SUMMARY OF THE INVENTION

According to the present invention we provide a titanium base alloy consisting of 5.0-7.0% aluminium, 2.0-7.0% zirconium, 0.1-2.5% molybdenum and 0.01-10.0 germanium and optionally one or more of the following elements: tin 2.0-6.0%, niobium 0.1-2.0%, carbon 0.02-0.1% and silicon 0.1-2.0%; the balance being titanium apart from incidental impurities.

The aluminium content may be in the range 5.0-6.0% or 5.0-6.5%.

The zirconium content may be in the range 2.0-4.0%, 2.0-6.0% or 3.0-7.0%.

## DESCRIPTION OF THE PREFERRED EMBODIMENT

Examples of an alloy according to the invention are now provided.

The alloys set out in Table 1 below were prepared:

TABLE 1

| ALLOY | Al   | Analysed Compositions (wt %) |     |     |      |      |     | Si  | Ge |
|-------|------|------------------------------|-----|-----|------|------|-----|-----|----|
|       |      | Sn                           | Zr  | Nb  | Mo   | C    |     |     |    |
| No. 1 | 5.78 | 4.0                          | 3.5 | 0.7 | 0.48 | 0.08 | 0.2 | 1.1 |    |
| No. 2 | 5.79 | 4.0                          | 3.5 | 0.7 | 0.49 | 0.08 | 0.2 | 0.6 |    |
| No. 3 | 5.88 | 4.0                          | 3.5 | 0.7 | 0.48 | 0.07 | 0   | 2.0 |    |

The prepared alloys were then each heat treated at 1030° C. for 2 hours and then air cooled. Subsequently each alloy was aged by heating at 700° C. for 2 hours. The mechanical properties for each alloy are set out in Table 2 below. The creep exposure was 100 hours at 600° C. at 125 MPa for each sample.

TABLE 2

| ALLOY | Test | TPS<br>Nmm <sup>-2</sup> | Mechanical Properties for 700° C. Age |                                 |                          |                 |    | Red.<br>Area<br>% |
|-------|------|--------------------------|---------------------------------------|---------------------------------|--------------------------|-----------------|----|-------------------|
|       |      |                          | 0.1%<br>YS<br>Nmm <sup>-2</sup>       | 0.2%<br>YS<br>Nmm <sup>-2</sup> | UTS<br>Nmm <sup>-2</sup> | Elongation<br>% |    |                   |
| No 1  | A    |                          | 990                                   | 1030                            | 1164                     | 10              | 18 |                   |
|       | B    |                          | 286                                   | 342                             | 551                      | 66              | 86 |                   |
|       | C    | 0.102                    | 1044                                  | 1059                            | 1041                     | 1               | 2  |                   |
| No 2  | A    |                          | 972                                   | 1002                            | 1125                     | 9               | 15 |                   |
|       | B    |                          | 329                                   | 355                             | 532                      | 40              | 71 |                   |
|       | C    | 0.124                    | 1022                                  | 1038                            | 1125                     | 1½              | 3  |                   |
| No 3  | A    |                          | 1033                                  | 1069                            | 1196                     | 8               | 16 |                   |
|       | B    |                          | 373                                   | 414                             | 583                      | 55              | 71 |                   |
|       | C    | 0.104                    | 1093                                  | 1107                            | 1111                     | 1               | ½  |                   |

TPS = Total Plastic Strain

YS = Yield Stress

The molybdenum content may be in the range 0.1-0.6%, 0.25-0.75% or 2.0-2.5%.

The germanium content may be in the range 0.01-5.0%, 0.01-0.2%, 0.01-0.5%, 0.1-2.0% or 2.0-5.0%.

More particularly, the alloy may consist of 5.3-6.1% aluminium, 3.5-4.5% tin, 3.0-4.0% zirconium, 0.5-1.0% niobium, 0.2-0.7% molybdenum, 0.1-0.5% silicon, 0.03-0.10% carbon and 0.3-3.0% germanium, the balance being titanium apart from incidental impurities.

Alternatively, the alloy may consist of 5.3-6.1% aluminium, 3.5-4.5% tin, 3.0-4.0% zirconium, 0.5-1.0% niobium, 0.2-0.7% molybdenum, 0.03-0.10% carbon and 0.3-3.0% germanium, the balance being titanium apart from incidental impurities.

Alternatively, the alloy may consist of 5.6-6.0% aluminium, 3.5-4.5% tin, 3.0-4.0% zirconium, 0.6-0.8% niobium, 0.3-0.6% molybdenum, 0.03-0.10% carbon, 0.15-0.5% silicon and 0.5-2.5% germanium, the balance being titanium apart from incidental impurities.

Alternatively, the alloy may consist of 5.6-6.0% aluminium, 3.5-4.5% tin, 3.0-4.0% zirconium, 0.6-0.8% niobium, 0.3-0.6% molybdenum, 0.03-0.10% carbon and 1.0-3.0% germanium, the balance being titanium apart from incidental impurities.

The alloys according to the invention are preferably heat-treated and subsequently cooled. The alloys are then preferably aged by heating to a selected temperature for a predetermined period of time and then cooled. The aging temperature may be in excess of 600° C. and may be as high as 700° C.

Test A was at room temperature; Test B was at an elevated temperature of 700° C.; Test C was at room temperature after the creep exposure referred to above.

The increase in yield stress for these alloys aged at 700° C. shows significant improvements over a comparable alloy containing silicon but with no germanium.

The alloys in accordance with the invention possess excellent creep resistance particularly at temperatures above 540° C. which makes them particularly valuable in gas turbine engine applications.

I claim:

1. A titanium base alloy consisting of 5.0-7.0% aluminium, 2.0-7.0% zirconium, 0.1-2.5% molybdenum and 0.01-10.0 germanium and optionally one or more of the following elements: tin 2.0-6.0%, niobium 0.1-2.0%, carbon 0.02-0.1% and silicon 0.1-2.0%; the balance being titanium apart from incidental impurities.

2. A titanium base alloy as claimed in claim 1 in which the aluminium content is in the range 5.0-6.0% or 5.0-6.5%.

3. A titanium base alloy as claimed in claim 1 or claim 2 in which the zirconium content is in the range 2.0-4.0%, 2.0-6.0% or 3.0-7.0%.

4. A titanium base alloy as claimed in claim 1 in which the molybdenum content is in the range 0.1-0.6%, 0.25-0.75% or 2.0-2.5%.

5. A titanium base alloy as claimed in claim 1 in which the germanium content is in the range 0.01-5.0%, 0.01-0.2%, 0.01-0.5%, 0.1-2.0% or 2.0-5.0%.

6. A titanium base alloy as claimed in claim 1 in which the alloy consists of 5.3-6.1% aluminium, 3.5-4.5% tin, 3.0-4.0% zirconium, 0.5-1.0% niobium, 0.2-0.7% mo-

lybdenum, 0.1-0.5% silicon, 0.03-0.10% carbon and 0.3-3.0% germanium, the balance being titanium apart from incidental impurities.

7. A titanium base alloy as claimed in claim 1 in which the alloy consists of 5.3-6.1% aluminium, 3.5-4.5% tin, 3.0-4.0% zirconium, 0.5-1.0% niobium, 0.2-0.7% molybdenum, 0.03-0.10% carbon and 0.3-3.0% germanium, the balance being titanium apart from incidental impurities.

8. A titanium base alloy as claimed in claim 1 in which the alloy consists of 5.6-6.0% aluminium, 3.5-4.5% tin,

3.0-4.0% zirconium, 0.6-0.8% niobium, 0.3-0.6% molybdenum, 0.03-0.10% carbon, 0.15-0.5% silicon and 0.5-2.5% germanium, the balance being titanium apart from incidental impurities.

9. A titanium base alloy as claimed in claim 1 in which the alloy consists of 5.6-6.0% aluminium, 3.5-4.5% tin, 3.0-4.0% zirconium, 0.6-0.8% niobium, 0.3-0.6% molybdenum, 0.03-0.10% carbon and 1.0-3.0% germanium, the balance being titanium apart from incidental impurities.

\* \* \* \* \*

15

20

25

30

35

40

45

50

55

60

65